

May 30, 1944.

G. J. BECKWITH

2,349,843

ELECTROLYTIC TREATMENT OF CHROMIUM ALLOYS

Filed June 14, 1941



Inventor:

GLENWOOD J. BECKWITH,

by: *John E. Jackson*  
His Attorney.

## UNITED STATES PATENT OFFICE

2,349,843

ELECTROLYTIC TREATMENT OF  
CHROMIUM ALLOYS

Glenwood J. Beckwith, Brecksville, Ohio, assignor to The American Steel and Wire Company of New Jersey, a corporation of New Jersey

Application June 14, 1941, Serial No. 398,160

3 Claims. (CL 204—140)

The demand for highly lustrous iron alloys of the class known as "stainless" or "rustless" steels is increasing daily, owing to the increasingly widespread use of such materials as ornamental and sanitary finishes and fittings in innumerable applications of stainless steel. However, in general, the production of the requisite lustrous finish to meet popular demand is attended with considerable difficulty.

At the time when stainless steel was introduced generally on the market, a good metal surface, which has been whitened by pickling, was the only material that was available practically. But as a use of such steels increased, there arose a demand for highly lustrous surfaces, which, because of their appearance, became utilized in both ornamental and utilitarian adaptations. In order to effect the production of demanded finishes, the articles were subjected to mechanical grinding, polishing and burnishing.

As the demands for products of this character increased, however, such mechanical procedures became too slow to fulfill the requirements. Consequently, investigators turned to chemical and then to electrochemical means, for producing the desired surface finish.

Chemical methods, while producing finished surfaces satisfactory for many purposes, nevertheless proved to be equally inferior to the finishes produced by mechanical operations. Additionally, control of chemical procedures is difficult, owing to variations in composition and character of the metal being treated, inherent irregularities in the surface, and many other factors which render a chemical treatment inconsistent in its effects.

Electrochemical methods have been tried with success, the procedure being to make the article being polished the anode in an electrolytic cell wherein the electrolyte may be any one of a variety of polishing solutions adapted for the purpose, or a mixture of various components intended to have a brightening action on the anode during electrolysis.

However, wide varieties of alloys are classed under the general heading of "stainless" or "rustless" steel. Some of these contain substantial amounts of nickel, while others are substantially straight chromium-iron alloys.

Additionally, the adaptation of such compositions in the form of round wires for the production of refrigerator shelves and other applications is becoming of increasing importance, with the attendant necessity of obtaining a uniform

bright polish on the round wires which make up these articles.

As has been indicated above, steels of this character may contain substantial amounts of nickel in addition to chromium, or, the nickel may be omitted and the percentage of chromium increased to give the straight rustless chromium steels.

Since nickel is a strategic metal with quantities thereof not sufficient, generally speaking, to fulfill defense requirements in national emergencies, under such conditions attention becomes placed more concentratedly upon the straight chromium-iron alloys, which are the materials being found customarily as round wires in refrigerator, and other, shelves, as well as various other applications wherein stainless steel is employed.

In view of the difference in composition, many procedures which are satisfactory in the case of the nickel containing stainless steels are not satisfactory for straight rustless chromium steels.

The present invention provides an improved process for electropolishing straight chromium rustless steels in whatever form, being adapted equally to the polishing of flat shapes as well as round wires or any other specific shape of metal.

In general, it has been found that stainless steels may be polished by making them an anode in a bath containing phosphoric acid, although other reagents may be utilized as an electrolyte. Thus, the electrolyte may be a highly concentrated solution of sulphuric acid, or chromic acid, or phosphoric acid, or mixtures of sulphuric and phosphoric acids, sulphuric acid and certain organic acid such as citric acid, or sulphuric and hydrofluoric acids. Phosphoric acid electrolytes have certain advantages as to economy and ready control of reactive properties, the usual electrolyte being composed of a concentrated aqueous solution of orthophosphoric acid.

It is well known that electrolytes are more conductive at elevated temperatures than they are at room temperatures, and in order to avoid an undulated or pitted surface, considerable care must be exercised in the matter of concentrations, current densities and other factors, particularly where stronger acids may be employed. Orthophosphoric acid appears to give the best results with the least attention as to control of conditions in the electrolyte.

Also, it is well known that certain organic materials serve to inhibit pitting by polarization phenomena, as is true, for example, in the chemical pickling of steels, but it is found that

such materials do not operate in this way in the presence of an electrolyzing current with the treated article as an anode in the bath.

In accordance with the present invention, it is found that a very satisfactory electrolyte is obtained by introducing small amounts of fluorescein in the electrolyte, particularly where straight chromium rustless steels are being treated.

In practice it is found that the optimum bath composition and its characteristics of operation are as follows:

*Bath composition by weight*

|                                  | Per cent | 15 |
|----------------------------------|----------|----|
| Orthophosphoric acid (85% grade) | 81.9     |    |
| Sulphuric acid (60° Baumé)       | 17.7     |    |
| Alcohol                          | .37      |    |
| Fluorescein                      | .03      |    |

In preparing the bath, the alcohol and fluorescein are mixed separately and a small amount of acid is added to it. It is then mixed into the main electrolyte.

The optimum conditions of electrolysis using the foregoing bath composition are as follows:

Current density 4 amps. per square inch  
Voltage 5 to 6 volts  
Temperature 140-160° F.  
Time 25 5 to 7 minutes (depending on

30 surface conditions)  
Results 35 A very bright and lustrous finish especially on cold drawn straight chromium rustless steel round wire containing 17% chromium.

The above bath operates more smoothly without the sulphuric acid but the finish is not nearly so bright. A content of more than 20% of 60° Baumé sulphuric acid severely pits both 17% and 12% straight chromium steel round articles even at increased current density.

Low current densities accompanied by low voltages are conducive to iron solution in preference to chromium, and a medium current density, for example, 4 amps. per square inch passivates or polarizes the iron areas so that a uniform dissolution of the surface is realized.

The temperature is found to be best kept within the limits specified above, since too high a temperature tends to pit the stock, and too low a temperature is not conducive to a brilliant luster.

That the presence of alcoholic fluorescein in the bath changes the polishing characteristics of the bath is discernible by the fact that some foaming is noticed and a decidedly different appearance of the polished surface results after adding the alcoholic fluorescein.

It is noticed in the practice that if straight fluorescein is added to the phosphoric acid, the luster of the stock is not greatly enhanced, and if sulphuric acid is added to the foregoing bath, the luster is improved only slightly and the degree of pitting is greater. But, on the other hand, if the fluorescein is dissolved in alcohol and then is added to the phosphoric acid as alcoholic fluorescein, the addition being made prior to the sulphuric acid addition, the stock is rendered to be about twice as lustrous as otherwise.

The accompanying drawing illustrates a diagrammatic sectional elevation of an apparatus for carrying out the present invention.

In the single view of the drawing, the article 2 to be polished is hung into the bath 4 on a hook or clamp 6 capable of carrying the current required. The bath 4 is contained in a suitable con-

20 tainer 8, which may be composed of acidproof brick, or other suitable material.

The article 2 forms an anode and its suspending hanger 6 engages a copper bus-bar 10 which is connected by current lead 11 to the positive terminal 12 of a suitable current generator 14.

Cathodes 16 of suitable material are spaced properly around the article 2, these cathodes being connected through bus-bars 18 and leads 20, 22, 23 to the negative terminal 24 of the generator 14, which for convenience is shown as being mounted on a shelf projecting from the cell.

The bus-bars form permanent connections and are conveniently located above the level of the electrolyte to avoid excessive action of electrolyte spray thereon.

In operating, it is highly important that a uniform flow of current be obtained from all parts of the surface, in order to avoid shaded or undulated areas.

Also, the hanger 6 is designed to assure an even distribution of current over the entire area of the anode 2 being polished. The hanger 6 is insulated in all parts exposed to the bath except on the area making intimate contact with the article being polished in order to prevent dissolution of the hanger and wastage of current.

It will be understood, of course, that the invention is not limited to the use of a phosphoric acid bath, or a mixture of phosphoric acid and sulphuric acid, containing alcoholic fluorescein as has been preferentially expressed herein, it having been found that, generally speaking, the presence of alcoholic fluorescein in any of the electrolytes used customarily for electropolishing stainless steels has a beneficial effect.

It will be understood that the foregoing composition of the bath as stated above, is the preferred composition which produces best results. However, the specific composition may range, in the completed electrolyte, from 80% to 90% of orthophosphoric acid (85% grade), from 10% to 20% of sulphuric acid of 60° Baumé grade, and appreciable amounts of alcoholic fluorescein, but less than 1% thereof.

It is found in practice that, however, in the case of straight chromium rustless steels, the preferred electrolyte avoids any appearance of blueness or fogging on the surface, but produces a mirror-like uniform finish at low cost both for material and current consumption.

It will be understood that the indicated percentages of components of the bath as given in the claims are percentages by weight in each instance.

55 I claim:

1. The process of producing highly polished surfaces on corrosion-resistant chromium steels, which consists in making the steel an anode in a bath containing approximately 81.9% by weight 60 of orthophosphoric acid of 85% grade, 17.7% of sulphuric acid of 60° Baumé gravity, .37% by weight of ethyl alcohol and .03% of fluorescein, the balance being essentially water, the fluorescein having been added to the bath as a solution thereof in the alcohol prior to addition of sulphuric acid to the bath, providing suitable cathodes to assure uniform current flow from all parts of the steel anode, maintaining the electrolyte at temperatures between about 140° to about 160° F. and passing a current through the resulting cell at a current density of substantially 4 amps. per square inch of anode surface and a voltage of from about 5 to about 6 volts.

2. The process for producing highly polished surfaces on corrosion-resistant chromium steels,

which consists in making the steel an anode in an aqueous electrolyte consisting of from 80% to 90% by weight of orthophosphoric acid of 85% grade, from approximately 10% to approximately 20% by weight of sulphuric acid of 60° Baumé, .37% by weight of ethyl alcohol and .03% by weight of fluorescein, the balance being essentially water, the fluorescein having been added to the bath as a solution thereof in the alcohol and prior to addition of sulphuric acid to the bath, providing suitable cathodes to assure uniform current flow from all parts of the steel anode, and passing a current through the resulting cell of sufficient den-

sity and for a sufficient length of time to effect a polish on the said metal surface.

3. An electrolyte for use in the anodic polishing of stainless steel, consisting of an aqueous solution containing in the finished solution, between 80% and 90% by weight of orthophosphoric acid of 85% grade, between 10% and 20% by weight of sulphuric acid of 60° Baumé, and .03% by weight of fluorescein dissolved in ethyl alcohol 10 amounting to .37% by weight of the electrolyte, the balance of the electrolyte being water.

GLENWOOD J. BECKWITH.